

July 7, 1925.

1,544,579

H. A. HERR

ELECTROTYPE PLATE

Filed March 17, 1924



Inventor  
Henry A Herr  
By *Joe Jochum Jr* Atty

Patented July 7, 1925.

1,544,579

# UNITED STATES PATENT OFFICE.

HENRY A. HERR, OF CHICAGO, ILLINOIS.

## ELECTROTYPE PLATE.

Application filed March 17, 1924. Serial N 699,794.

*To all whom it may concern:*

Be it known that I, HENRY A. HERR, a citizen of the United States, residing at Chicago, in the county of Cook and State of Illinois, have invented certain new and useful Improvements in Electrotype Plates, of which the following is a specification.

In electrotype processes it is necessary to employ plates having a very hard surface and for that reason electrotype plates are usually constructed of copper owing to the hardness of the material, with the result that a printing surface which is quite durable will be produced. These copper plates, however, after a number of impressions have been taken therefrom, wear out, often-times before the completion of the job, particularly if a great many copies are pulled or taken therefrom.

It is one of the objects of the present invention to increase the life of a copper electrotype plate by increasing the hardness of the printing surface thereof.

By actual test it has been found that the life of a plate of this character which has been treated in accordance with the present invention has been increased to such an extent that substantially five times as many more copies or impressions have been obtained therefrom than from the ordinary or usual copper faced electrotype plate which has not been treated according to this invention.

In the drawing the figure is a sectional view on an enlarged or exaggerated scale of an electrotype plate prepared in accordance with the principles of this invention, the numeral 10 designating the electrotype plate proper and 11 designates a coating of iron solution deposited upon the printing surface thereof.

Any suitable iron solution may be em-

ployed but in practice a solution consisting of sixteen ounces of sulphate of iron; eight ounces of ammonia; one ounce of boric acid, to which is added a sufficient quantity of water to produce one gallon of the solution, has been employed with efficient results.

In use the copper plate is first cleaned and the iron solution is then deposited upon the surface of the plate by any suitable and well-known electrolytic process, after which the plate will then be ready for use.

In practice it has been found that some of the inks contain certain chemicals and ingredients which attack or eat the copper of the plate, but with a plate of this character having an iron coating thereon in accordance with this invention, such attacks upon the plate are resisted and the life of the plate will be materially increased. Furthermore the cost of producing or treating a plate with this solution will not be materially increased.

What is claimed as new is:—

1. A copper electrotype plate having its printing surface coated with iron.
2. A copper electrotype plate having a deposit of iron upon its printing surface.
3. A copper electrotype plate having an iron printing surface.
4. The method of preparing a copper electrotype plate by coating the printing surface thereof with a deposit of iron.

5. The method of preparing a copper faced electrotype plate by depositing iron upon the printing surface thereof by electrolytic process.

In testimony whereof I have signed my name to this specification, on this 14th day of March, A. D. 1924.

HENRY A. HERR.